# EUROPEAN PATENT SPECIFICATION

(11) **EP 0 159 120 B1**
(45) Date of publication and mention of the grant of the patent: **29.04.1987**
(21) Application number: 85301398.5
(22) Date of filing: 28.02.1985
(51) Int. Cl.: D01F 9/22, D01F 9/14

(54) **Lubricating agents for use in the production of carbon yarns**
Schmiermittel und deren Anwendung bei der Herstellung von Karbonfasern
Agents lubrifiants et leur utilisation dans la fabrication de fibres de carbone

(30) Priority: 29.02.1984 JP 39541/84
(43) Date of publication of application: 23.10.1985
(73) Proprietor: Takemoto Yushi Kabushiki Kaisha, Gamagouri-shi Aichi-ken (JP)
(72) Inventor: Fujii, Tsukasa, Toyota-shi Aichi-ken (JP); Isobe, Jun, Toyohashi-shi Aichi-ken (JP)
(74) Representative: Ablewhite, Alan James

## Description

### Background of the Invention

This invention retates to lubricating agents for the production of carbon yarns and more particularly to lubricating agents having specified amino polysiloxanes as effective component. When applied to acrylic fibers or carbon fibers derived from pitchy material to be used as a precursor for the infusibilizing process (hereinafter to be referred simply as precursor), these agents can not only give to the precursor a superior filament separabitity and processability, but also prevent adhesion after the infusibilizing process, thus making it possible to produce carbon yarns with superior physical chacacteristics.

Carbon yarns are generally produced by first obtainind non-flammable yarns from a precursor by a process (hereinafter referred simply as the infusibilizing process) wherein the precursor is heated and burnt at 200 - 3000C in an oxidizing atmosphere; and second by a carbonization process wherein carbonization takes place in an inert atmosphere at a high temperature. e.g. over 700°C. In such a case, a lubricating agent is applied prior to the infusibilizing process, and usually during the process in which the precursor itself is produced. In addition to the generally desired charactecistics such as lubricity, antistatic capability and cohesion, however, it is important, in view of the aforementioned processes for the production of carbon yarns, that the lubricating agent to be used for this purpose be superior to providing a good filament separability and infusibility.

In the past, various substances, including phosphates of alkati metals, various cationic activators, polyoxyalkylene ether, etc.. have been used as lubricating agents of this type. Although they are generally acceptable regarding antistatic capability, cohesion and lubricity, they are inferior regarding their filament separabitity because of their basic tendency to become decomposed. In addition, they have the disadvantage of generating tar during the infusibilizing process or of vaporizing mostly during the initial heating period and causing adhesion between the fibers.

In order to overcome this difficulty, many silicone-type lubricating agents have been considered such as dimethyl polysiloxanes, phenylmethyl polysiloxanes, epoxy polysiloxanes, polyether polysiloxanes, amino polysiloxanes, etc. (Japanese Patents Tokko 51-12739, Tokko 52-24136, Tokkai 52-148227, etc.). These siticone- type lubricating agents, however, have various disadvantages. Dimethyl polysiloxanes and phenylmethyl polysiloxanes are thermally superior but provide poor filament separability in the precursor and are poor in prevention of adhesion in the infusibilizing process. This may be because they do not contain polar groups in their molecules and hence their orientation (hereinafter used to mean the characteristic of uniform adhesion) regarding the precursor is insufficient. Moreover, since they are non-polar, problems of fuzz and yarn breakage caused by static electricity can occur easily.

Epoxypolysiloxanes tend to cause fiber-to-fiber fixing due, for example, to the ring-opening polymerization of epoxy groups within their molecules and since they themselves generate tar, they are totally incapable of preventing mutual adhesion during the infusibitity process. Their presence, therefore, makes the problem worse instead of solving it. As for polyether polysiloxanes, the ether bonds within, their molecules are thermally weak so that they mostly become decomposed and diffuse away, failing to exercise their capability of preventing adhesion. Moreover, their heat of thermal decomposition becomes a cause of abnormal reactions involving the yarns.

Amino polysiloxanes of the type proposed in the past, although they have more favorable characteristics than the other conventional silicone type lubricating agents discussed above have only one nitrogen atom per amino-modified group within their molecules and this means that only weak polar groups are loosely distributed around. Accordingly their orientation capability with respect to the precursor is inferior and the filament separability and degree of adhesion prevention they provide are not sufficient to be satisfactory.

It is therefore an object of this invention to eliminate the aforementioned disadvantage by providing lubricating agents which are superior in processability and opening property of each filament in the subsequent processes, including the production of precursors and the infusibilizing process, without causing problems such as adhesion. and thus make it possible to produce high quality carbon yarns.

The above and the other objects of the present invention have been achieved by the present inventors with the discovery that good lubricating agents for this purpose have as an effective component amino polysiloxans with specific amino-modified groups of a certain nitrogen content.

### Detailed Description of the Invention

According to this invention there is provided a lubricating agent for the production of carbon yarns characterised by comprising at least one amino polysiloxane of the general formula (I) as an effective component, the nitrogen content of said effective component being 1 weight % or less: where A is
X represents an alkylene group with 3 to 5 carbon atoms,
Y represents an alkylene group with 2 to 8 carbon atoms
or a phenylene group, R, and R₃ each represent a hydrogen atom, an alkyl group with 1 to 5 carbon atoms
or a phenyl group, R₂ and R₄ each represent methyl
or ethyl groups, R₅, R₆ and R₇ each represent a hydrogen atom, a methyl group or an ethyl group,
n is an integer equal to or greater than 1 and p is 0 or an integer in the range of 1 to 5.

Amino polysiloxanes of formula (I) may be obtained, for example, by condensation of a silane containing an amino group and a diorgano polysiloxane with terminal hydroxyl groups. In this situation, both a single system of amino polysiloxanes shown by (I) and a mixed system of aforementioned amino polysiloxane and a polysiloxane-type compound corresponding to A - OH in (I) can be obtained. depending on the molar ratio between silane containing the amino group and the diorgano polysiloxane with terminal hydroxyl groups. Both these systems contain amino polysiloxanes shown by (I) as effective component and hence are lubricating agents according to the present invention but it is a requirement that the nitrogen content of said effective component be 1 weight% or less. If the nitrogen content of the effective component exceeds 1 weight%, the orientation characteristic regarding the precursor becomes improved but the heat resistance becomes worse and tar comes to be generated during the infusibilizing process so the ability to prevent adhesion is significantly affected. The viscosity of the effective component at 25°C should preferably be 1-100 cm²/s (100 to 10.000 cst (centistokes)) and its nitrogen content should preferably be 0.5 weight% or less. This is chiefly in anticipation of situations where diffusion may lower the capability of preventing adhesion and an increase in viscosity may adversely affect lubricity. In these cases, however, good results can generally be obtained if a mixed system of the af orementioned type is used.

The lubricating agents of the present invention may be used together with any known lubricant, softening agent, antistatic agent, surface active agent, antioxidant, antiseptic or conventional lubricating agent for the production of carbon yarns, as long as the desired effects of the present invention are not adversely affected. There is no limitation on the amount of the aforementioned effective component to be contained, but it should preferably be 40 weight% or greater in view of the required filament separability of the precursor and the required adhesion-preventing property during the infusibilizing process.

The lubricating agents of the present invention are applied during the precursor production process or before the infusibilizing process. As for the mode of application, they may be applied either as an emulsion, as a solution with an organic solvent or straight. The may be applied by a kiss-roll method, a spray method or a guide-oiling method. The amount to be deposited in these cases is preferably 0.01 to 5 weight% with respect to the precursor in order to obtain the required effects fully but economically.

As explained above, the lubricating agents of the present invention containing amino polysiloxanes shown-. by (1) as the effective component have a superior processability in the precursor production process and the infusibilizing process and in particular provide superior filament separability in the precursor and a superior capability of preventing adhesion in the infusibilizing process so that they can show better results than the previously proposed types of amino polysiloxanes. It is not clear why this result is obtained, but amino polysiloxahes of the present invention are clearly different in that they contain amino-modified groups at both ends of their molecules, it may be concluded that amino polysiloxanes of the present invention are more strongly oriented with respect to the precursor, possibly as a result of the aforementioned difference, and that the extent of this orientation property becomes particularly important when the nitrogen content is reduced in view of the required heat resistance characteristics.

The following test examples are described by way of illustration of the present invention and its effects and do not comprise a limiting definition of the present invention.

### Test Examples

Water emulsions of lubricating agents comprising 85 weight % of the processing agents shown in Table 1 and 15 weight % of POE nonylphenyl ether were prepared. Test yarns were prepared by applying these water emulsions to acrylic filament yarns (83 dtex/40 filaments) so that 0.5 ± 0.1 weight % will be deposited on each by the kiss roll method, and the coefficients of friction and generation of static electricity were measured and evaluated by the method to be described.

In addition, the aforementioned water emulsions were applied to acrylic filament yarns (17776 dtex/12000 filaments) at the rate of 0.5 ± 0.1 weight % by immersion method. The yarns were then dried for 4 seconds at 115°C by means of a dry heat roller to prepare a precursor tow and this was used as sample to evaluate the filament separability by the method described below.

Furthermore, the precursor tow was processed for 60 minutes inside an oven of forced circulation type at 240°C to obtain infusibilized fibers and they were used as samples to evaluate their infusibility by the method to be described later.

### Measurement of the coffecient of friction

The sample was left for 24 hours under the condition of 20°C and 65%RH and caused to run in contact with a cylindrical chromium-plated pin under the same conditions with initial tension 20 g and yarn velocity of 100m/min. Coefficient of friction was measured by using a γ-meter (made by Eiko Sokki-sha). The lower the measured value. the better is the result.

### Evaluation of static electricity

Concurrently with the aforementioned measurement of coefficient of friction, electrostatic voltage of the yarn after the contact with the chromium-plated pin was measured by means of a static electrometer (made by Kasuga Denki Kabushiki Kaisha) and the results were evaluated according to the following standards:
0: Voltage less than 100V
1: Voltage 100V to less than 300V
X: Voltage 300V or greater

### Filament Separability

The sample was cut to 2cm lengths and shaken lightly over a black sheet of paper and its filament separability was evaluated according to the following standards:
00 : Separability very good
0: Good
1: Bad
X: Very bad

### Infusibility

The sample was cut to 2cm and shaken lightly over a white sheet of paper and its infusibility was evaluated according to the following standards:
00: No fusion
0: Very little fusion
1 : Some fusion
X: Fusion to a considerable degree

The results are shown in Table 1. One can clearly see from these results that the lubricating agents of the present invention provide superior filament separability and infusibility which are necessary properties of any lubricating agent for the production of carbon yarns, in addition to other superior characteristics such as lubricity, antistatic capability etc.

Amino polysiloxane (A):
Amino polysiloxane (B): and
   Coe = Coefficient of friction
   Vol = Evaluation of electrostatic voltage
   Sep = Evaluation of filament separability
   Inf = Evaluation of infusibility

## Claims

1. A lubricating agent for use in the production of carbon yarns, characterised in that it comprises at least one amino polysiloxane of formula (I) where A is
X represent an alkylene group with 3 to 5 carbon atoms,
Y represent an alkylene group with 2 to 8 carbon atoms
or a phenylene group, R₁ and R₃ each represent a hydrogen atom, an alkyl group with 1 to 5 carbon atoms or
a phenyl group, R₂ and R₄ each represent a methyl group or an ethyl group, Rₛ, R₆ and R₇ each represent a hydrogen atom, a methyl group or an ethyl group, n is an integer equal to or greater than 1 and p is 0 or an integer in the range of 1 to 5, as effective component. the nitrogen content of said effective component being 1 weight% or less.

2. A lubricating agent according to claim 1, wherein the viscosity at 25°C of said effective component is 1 to 100 cm2/s (100 to 10000 cst) and the nitrogen content of said effective component is 0.5 weight% or less.

3. A lubricating agent according to claim 1 or claim 2. containing an effective component of formula (I) in which R₁, R₂. R₃ and R₄ all represent methyl groups.

4. A lubricating agent according to claim 3. containing an effective component of formula (I) in which R₇ and R₅ represent hydrogen atoms, p is zero, and X represents a propylene group.

5. A method of lubricating yarns used in the manufacture of carbon yarns, characterised in that it comprises applying thereto a lubricating agent according to any of claims 1 to 4.

## Revendications

1. Agent lubrifiant, pour utilisation dans la production de fils de carhone, caractérisé en ce qu'il comprend au moins un aminopolysiloxane de formule (I) dans laquelle A est
X représente un groupe alkylène ayant de 3 à 5 atomes de carbone,
Y représente un groupe alkylène ayant de 2 à 6 atomes de carbone ou un groupe phénylène, R, et R₃ représentent chacun un atome d'hydrogène, un groupe alkyle ayant de 1 à 5 atomes de carbone ou un groupe phényle, R₂ et R₄ représentent chacun un groupe méthyle ou un groupe éthyle, R₅, Rₛ et R₇ représentent chacun un atome d'hydrogène, un groupe méthyle ou un groupe éthyle, n est un entier supérieur ou égal à 1, et p vaut 0 ou est un entier dans l'intervalle de 1 à 5, en tant que constituant actif, la teneur dudit constituant actif en azote étant de 1 % en poids, ou moins.

2. Agent lubrifiant selon la revendication 1, dans lequel la viscosité à 25°C dudit constituant actif est de 1 à 100 cm²/s (100 à 10 000 cSt), et que la teneur dudit constituant actif en azote est de 0,5 % en poids ou moins.

3. Agent lubrifiant selon la revendication 1 ou la revendication 2, contenant un constituant actif de formule (I) dans laquelle R₁, R₂, R₃ et R₄ représentent tous des groupes méthyle.

4. Agent lubrifiant selon la revendication 3, contenant un constituant actif de formule (I) dans laquelle R₇ et R₅ représentent des atomes d'hydrogène, p vaut zéro, et X représente un groupe propylène.

5. Procédé de lubrification de fils utilisés dans la fabrication de fils de carbone, caractérisé en ce qu'il comporte l'application à ceux-ci d'un agent lubrifiant selon l'une quelconque des revendications 1 à 4.

## Patentansprüche

1. Ein Schmiermittel zur Anwendung bei der Herstellung von Karbonfasern, dadurch gekennzeichnet, daß es zumindest ein (1) Aminopolysiloxan der Formel (I) enthält. Dabei ist A
X stellt eine Alkylen-Gruppe mit 3 bls 5 Kohlenstoffatomen dar,
Y stellt eine Alkylen-Gruppe mit 2 bis 6 Kohlenstoffatomen dar oder aber eine Phenylen-gruppe, R₁ und R₃ sind jeweils ein Wasserstoffatom, eine Alkyl-Gruppe mit 1 bis 5 Kohlenstoffatomen oder eine Phenyl-Gruppe, R₂ und R₄ stehen jeweils für eine Methyl- oder eine Äthyl-Gruppe, R₅, R₆ und R₇ stellen jeweils ein Wasserstoffatom, eine Methyl- oder eine Äthyl-Gruppe dar, n ist ein Ganzes, das gleich oder größer ist als 1, und p ist entweder 0 oder ein Ganzes im Bereich von 1 bis 5, als Wirkstoffkomponente, wobei deren Stickstoffgehalt 1 Gewichtsprozent oder weniger beträgt.

2. Ein Schmiermittel gemäß Anspruch 1, bei dem die Viskosität der Wirkstoffkomponente bei 25 °C 1 bis 100 cm²/s (100 bis 10000 cSt) und der Stickstoffgehalt dieser Wirkstoffkomponente 0,5 Gewichtsprozent oder weniger betragen.

3. Ein Schmiermittel gemäß Anspruch 1 oder 2, das eine Wirkstoffkomponente der Formel (I) enthält, bei der R₁, R₂, R₃ und R₄ alle Methyl-Gruppen darstellen.

4. Ein Schmiermittel gemäß Anspruch 3, das eine Wirkstoffkomponente der Formel (I) enthält, bei der R₇ und R₅ Wasserstoffatome sind, p gleich null ist und X eine Propylen-Gruppe darstellt.

5. Ein Verfahren zum Schmieren von Fasern zur Anwendung bei der Herstellung von Karbonfasern, dadurch gekennzeichnet, daß bei diesen Fasern ein Schmiermittel gemäß einem der Ansprüche 1 bis 4 zum Einsatz kommt.
